

May 15, 1928.

1,669,580

M. SPEICHERT

PROCESS FOR EXTRACTING TIN MIXTURE FROM LEAD AND TIN ALLOYS

Filed Sept. 18, 1926

2 Sheets-Sheet 1

Fig. 1.



Inventor:  
Max Speichert.  
per  
*Rowatkin*  
Attorney.

May 15, 1928.

1,669,580

M. SPEICHERT

PROCESS FOR EXTRACTING TIN MIXTURE FROM LEAD AND TIN ALLOYS

Filed Sept. 18, 1926

2 Sheets-Sheet 2

Fig. 2.



Inventor:  
Max Speichert.  
per  
*R. W. K.*

Attorney.

## UNITED STATES PATENT OFFICE.

MAX SPEICHERT, OF BERLIN-TEMPELHOF, GERMANY.

## PROCESS FOR EXTRACTING TIN MIXTURE FROM LEAD AND TIN ALLOYS.

Application filed September 18, 1926, Serial No. 136,299, and in Germany October 11, 1924.

This invention relates to a process for extracting "tin mixture" from lead and tin alloys containing antimony and copper or one of these metals with or without small amounts of other metals, or for preparing bearing metals or the like free from lead or having only a small proportion thereof.

Liquation or segregation was hitherto resorted to as a means of extracting components from alloys or extracting alloys of dissimilar composition therefrom by melting the easily liquefied components out of the solid remaining residue of the initial material. This method of proceeding however has only a limited number of applications because the composition of the products thus obtained is not always as expected, chiefly for the reason that the temperature cannot be regulated with sufficient accuracy, the consequence being that the melted-out metal is not uniform in composition.

Furthermore, the old liquation process must be carried through several stages or steps in order to secure an alloy of fairly accurate composition.

The process of my invention overcomes these difficulties encountered in the liquation process by the substitution therefor of a single stage or step which corresponds to and yet is essentially different from the last step of the liquation process, and by which an alloy of accurate composition can be obtained.

I have found that it is possible to extract individual components or alloys of dissimilar but quite definite composition from metal alloys above referred to by first melting the whole of the alloy and thereafter slowly allowing it to cool. Certain components of the alloys crystallize individually or as a mixture while other components remain fluid and may be removed in that state from the melting furnace. For allowing the fluid portion to be drawn off the molten metal bath should have a certain depth to enable the solid and liquid portion to separate from each other well. This renders it possible to separate individual components or alloys of definite composition (more particularly eutectic mixtures having a definite melting point) by suitably regulating the temperature and selecting the composition of the charge.

Taking as an example an alloy of tin, antimony, lead and copper, as available in

scrap from bearing metal, melting the said alloy as just outlined and allowing it to cool slowly, antimony and copper reach the solid state while tin and lead with a practically negligible percentage of antimony and copper remain fluid. The liquid mixture forms the so-called "tin mixture" suitable as a main component of solder.

As another example, the initial material may be made up by mixing scrap of dissimilar composition so that tin and lead in the molten material are in proportion of their eutectic mixture. In this case there is a practically complete separation of the eutectic mixture of tin and lead with the exceedingly small percentage of antimony and copper, on the one hand, and of copper and antimony, on the other hand. The formation and removal of the eutectic mixture are of course not prevented by an excess of tin or lead, but the amount of metal in excess is lost as it solidifies with the antimony and the copper.

The above method of proceeding is likewise suitable for making bearing metals or the like free from lead or having only a small proportion thereof. To this end the charge must have an ample proportion of copper and a large excess of tin. Lead may thus be completely extracted by removing the mixture which contains the whole (or substantially the whole) of the lead and which remains fluid when the molten material cools down, leaving behind an alloy of tin, antimony and copper.

Other alloys containing lead and tin can be dissociated in a similar manner by making preliminary tests as regards composition of the charge and temperature to suit each particular case. It is however, necessary that the metals present besides lead and tin in the alloys or alloy mixtures used as starting materials have melting points above that of the eutectic mixture of lead and tin which may of course contain the minor quantities of other metals above referred to.

*Example 1, for making "tin mixture".*—A charge composed of 44% tin, 32% lead, 20% antimony and 4% copper is melted and allowed to cool to 182° C. The mixture of 55 parts of tin and 41.4 parts of lead, with an allowable proportion of 0.1 part of copper and 3.5 parts of antimony, remains fluid and is drawn off while the remaining antimony and copper are left behind in the solid state.

*Example 2, for making bearing metal poor in lead.*—A charge composed of 70% tin, 13% lead, 12% antimony and 5% copper is melted and allowed to cool to 182° C. Out of 100 parts of the charge 30 parts of "tin mixture" are obtained in the form of a fluid mixture (55 parts of tin and 41.4 parts of lead, with the allowable proportion of 0.1% copper and 3.5% antimony) and 70 parts of solid bearing metal are obtained, containing 10 76% tin, and 16% antimony, 7% copper and 1% lead.

The process can be carried out in a similar manner, if the starting material, besides lead and tin, contains instead of both antimony and copper, only one of these metals.

*Example 3.*—A charge composed of 46% tin, 34% lead and 20% antimony is melted and allowed to cool to 182° C. The mixture of 55 parts of tin and 41.4 parts of lead with the allowable proportion of 3.5 parts of antimony remains fluid and is drawn off, while the main quantity of antimony is left behind in the solid state.

25 The process just described can be carried out in reverberatory furnaces differing from the ordinary types of such furnaces only in that the dimensions, especially as regards depth of hearth, must be large enough to 30 allow the molten material to cool so slowly that the crystallizing components separate from those which remain fluid; in other words, the material must not solidify throughout.

35 The process may be carried out for example in a cylindrical furnace rotatable about its longitudinal axis, as commonly used for melting copper.

A furnace of this nature is illustrated in 40 Figure 1 in cross-section.

45 This furnace comprises a casing 1 with a lining 2 of refractory material. The end faces of the furnace have a heat-resisting wall 3 extending vertically along two-thirds of the said faces. A gas burner (not shown) is above the said wall at one end of the furnace, the products of combustion escaping at the other end. The material to be melted is introduced through a charging hole 4, 50 whereafter heat is applied until all the charge is melted. The supply of heat is now discontinued and the furnace is allowed to cool slowly. It cools on all sides so that a crystallized outer layer 5 is formed while 55 the centre or core 6 remains fluid. A pyrometer shows when the cooling reaches the desired point and a tap tube 7 (suitably extended into the interior of the furnace) is opened so that the said fluid centre or core 60 flows out by gravity since air is allowed to pass through the porous crystalline outer layer. The furnace is mounted on rollers 8 so that it may be tilted by means of a suitable gear for the purpose of completely 65 moving the fluid material.

The furnace shown in cross-section in Figure 2 has proved particularly suitable for carrying out the present process.

This furnace, preferably rectangular or circular in cross-section, comprises a hearth 70 made of fire-resisting material 9 and considerably deeper than in the usual reverberatory furnaces. The furnace is charged through an aperture 10 and heated by suitably located gas burners 11. In a furnace of 75 rectangular cross-section there is preferably one burner at the end of each wall, the nozzle of each burner being substantially parallel to the adjacent wall. A whirling flame is thus produced which comes uniformly in 80 contact with the whole of the surface of the charge. The products of combustion are discharged through a chimney 12.

The charge is allowed to cool after it has been melted. In this case it cools from the 85 surface, so that the crystallized components form an upper layer 13 while those that remain fluid are at 14 in the lower portion of the hearth. They can thus be drawn into a receptacle 16 through a tap hole 15. As 90 shown in the drawings, the floor of the hearth has surfaces inclined towards the tap hole.

What I claim is:—

1. A process for extracting, from lead and 95 tin alloys containing antimony and copper and which may contain small amounts of other metals, an alloy known as "tin mixture" and being a eutectic mixture containing from 54.5 to 55% of tin, not more 100 than 3.6% of antimony, not more than 0.2% of copper, the remainder being lead, said process consisting in melting immediately 105 as a whole, without any previous treatment such as liquation, the said starting alloys, cooling the molten material until only the 110 said mixture of lead and tin with only a slight percentage of antimony and copper remains fluid, and drawing off said fluid mixture.

2. A process for extracting, from lead and 115 tin alloys containing antimony and copper and which may contain small amounts of other metals, an alloy known as "tin mixture" and being a eutectic mixture containing from 54.5 to 55% of tin, not more than 3.6% of antimony, not more than 0.2% of copper, the remainder being lead, said process consisting in selecting said starting 120 alloys so that the lead and tin are in the proportions of the said eutectic mixture, melting said alloys, cooling the molten material until only a mixture of lead and tin with only a slight percentage of antimony and copper remains fluid, and drawing off said 125 fluid mixture.

3. The process for extracting "tin mixture" from lead and tin alloys containing antimony and copper and which may contain small amounts of other metals, in which al 130

loys the proportion of tin is such that practically all the lead is combined with tin to form therewith a eutectic mixture, there being enough tin left to form with the other metals including copper and antimony an alloy having the required composition for use as a bearing metal, which process consists in melting said alloys, cooling the molten material until only a mixture of lead

and tin with a practically negligible percentage of antimony and copper remains fluid, and separating the fluid "tin mixture" from the solid portion forming the bearing metal.

In testimony whereof I have affixed my signature.

MAX SPEICHERT.